

Patented Apr. 4, 1944

2,345,734

# UNITED STATES PATENT OFFICE

2,345,734

## SELF-EMULSIFYING PHOSPHATED AND PHOSPHITED OILS AS ANTISTATIC LUBRICANTS

Joseph B. Dickey and James G. McNally, Rochester, N. Y., assignors to Eastman Kodak Company, Rochester, N. Y., a corporation of New Jersey

No Drawing. Application July 18, 1939,  
Serial No. 285,208

7 Claims. (Cl. 8—142.5)

This invention relates to the preparation and use of dispersing agents in the compounding of compositions adapted for the lubrication and other treatment of filaments and yarns composed of or containing organic derivatives of cellulose such as cellulose acetate, cellulose propionate, cellulose acetate propionate and cellulose acetate butyrate.

As is well known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. It is also necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion," "pin holes," "laddering," and the like.

In the preparation of compositions for this purpose it is customary to employ as emulsifying agents metallic and organic soaps and water-soluble soaps or dispersing agents containing a sulphonic acid group. Notwithstanding the many materials which have been suggested as emulsifying or dispersing agents in the preparation of yarn treating emulsions, there is still a great demand in the textile industry for agents which will give stable aqueous emulsions of the textile lubricants commonly employed to lubricate and otherwise treat yarns composed of or containing organic derivatives of cellulose and similar cellulosic materials.

This invention has as its principal object to provide a new class of self-dispersible compounds which are particularly adapted for use as emulsifiers for textile yarn lubricants, as textile lubricants as such, and as deelectrifying or anti-static agents. A further object is to provide yarn lubricating formulas which can be readily removed from the yarns by the usual scour baths. A specific object is to provide a method for the preparation of phosphated and phosphited blown and unblown oils, fats and waxes. Another object is to provide an improved type of stable yarn lubricating emulsion in which emulsification is obtained by means of these phosphated and phosphited compounds. Other objects will appear hereinafter.

These objects are accomplished by the following invention which, in its broader aspects, comprises the discovery that by treating blown or oxidized drying or semi-drying oils and the

hydroxylated or unblown oils, fats, and waxes, such as castor oil, cod liver oil, rapeseed oil, carnauba wax and Japan wax with a phosphating agent such as phosphoric acid and the various pyro-phosphoric acids, thio-phosphoric acids and the corresponding pyro acids, phosphorus pentoxide, phosphorus pentasulfide, phosphorus pentachloride, phosphorus oxychloride, phosphorus thiochloride and the like, or with a phosphiting agent such as phosphorus acid, phosphorus trichloride, phosphorus oxide,  $P(OH)_2Cl$ ,  $P(OH)Cl_2$ ,  $PCl_2-NH_2$  and the like—self-dispersible compounds which are excellent emulsifiers for textile lubricants and also good lubricants in and of themselves, may be produced. Although all of the above-mentioned phosphating and phosphiting agents are operative to produce such compounds in accordance with our invention, phosphoric acid is probably the least efficacious. Of the various hydroxylated or unblown oils which we have found satisfactory for the purposes of our invention, the highly hydroxylated oils such as castor oil and cod liver oil are outstanding in their ability to give phosphated and phosphited compounds capable of acting as surface active, de-electrifying, emulsifying, and lubricating agents in accordance with our invention.

It should be noted that all of the oils within the contemplation of our invention are composed of or contain compounds having at least one free hydroxyl group or its equivalent, in its molecule which is subject to phosphorylation or phosphitation.

Of these various oils we have found that those resulting from the phosphorylation or phosphitation of vegetable, animal and marine oils having an iodine value between 50 and 100, and the organic and inorganic base salts of these phosphated and phosphited oils, are of exceptional value as surface-active, deelectrifying, emulsifying, and lubricating agents.

Of the many phosphated oils of our invention those which have proved outstanding in actual practice are phosphated blown neat's-foot, phosphated blown olive and phosphated blown castor oils. Of the phosphated unblown or hydroxylated oils, phosphated castor and cod liver oils are outstanding.

We have found that these phosphated and phosphited blown and unblown oils and in particular the inorganic and organic base salts of phosphated and phosphited blown oils having an iodine number of 50-100, are especially effective in the compounding of compositions adapted for the lubrication and other treatment of yarns composed of or containing organic derivatives of cellulose, such as cellulose acetate, since, not only are they excellent dispersing or emulsifying agents for the textile lubricants commonly em-

ployed in such compounds, for example, neat's-foot, olive, and light mineral oils, but also are themselves self-emulsifiable oils which may be used as the primary lubricant in such compositions. These phosphated and phosphited oils are also excellent de-electrifying or anti-static agents and may also be used as vehicles for fugitive dyes and as dye assistants in the permanent dyeing of various types of textile fabrics including those composed of cellulose acetate and other synthetic materials.

Our invention will be more readily understood by reference to the following examples in which we have set forth several preferred and typical methods of preparing the compounds of our invention as well as several typical and preferred methods of the application of such compounds to cellulose derivative yarns, these examples being included merely for purposes of illustration and not as a limitation of the invention.

#### PHOSPHATED COMPOUNDS

##### Example 1

37 gm. of castor oil are added to 6 gm. of  $\text{POCl}_3$  in pyridine. The reaction is completed by warming. The product is filtered, washed with aqueous bicarbonate, and neutralized. The reaction product is a self-dispersible, cloudy, brown oil.

##### Example 2

200 gm. of rapeseed oil are warmed with 25 gm. of



in pyridine. The reaction product is filtered and the pyridine is removed in a vacuum. The solution is neutralized with aqueous ethylamine to give a pleasant smelling viscous yellow oil.

##### Example 3

Carnauba wax and crystalline phosphoric acid are heated in a molecular proportion of 1:1 on the steam bath for 24-60 hr. The product, after neutralization with a suitable base such as diethylcyclohexylamine, triethanolamine, tetraethylammonium hydroxide, ditetrahydrofurylamine, etc., is a self-dispersible, gelatinous dark oil.

##### Example 4

A mixture of 75 gm. of castor oil and 25 gm. of carnauba wax is treated with 75 gm. of ethylene glycol and 20 gm. of  $\text{P}_2\text{O}_5$ . The reaction product is neutralized with 90% triethanolamine. The heavy brown oil obtained is self-emulsifiable in water.

##### Example 5

100 gm. of reduced and partially acetylated castor oil are heated with 60 gm. of sirupy phosphoric acid and 20 gm. of  $\text{P}_2\text{O}_5$  for 10 hr. at 60°. The neutralized product is an oily solid.

##### Example 6

200 gm. of Japan wax are heated with 250 gm. of  $\text{PSCl}_2$  ( $\text{NH}_2\text{C}_1\text{H}_{35}$ ) and 50 gm. of Cellulosolve for 10 hr. in 1 liter of  $\text{CCl}_4$ . The reaction is completed by removing the  $\text{HCl}$  and  $\text{CCl}_4$  in vacuo. The product is a low melting waxy solid.

##### Example 7

100 gm. of castor oil are heated in vacuo at 180° with 100 gm. of anhydrous  $\text{Na}_2\text{HPO}_4$ , using

glycerine as a solvent. The reaction product is washed with a small quantity of water, leaving a slippery waxy powder.

##### Example 8



10 are ground with 4 lb. of phosphated castor oil, prepared as described above, and the mixture poured into hot water. 500 lb. of cellulose acetate thread, filaments, fiber or cloth are then dipped and dyed.

##### Example 9

15 100 gm. of phosphated carnauba wax are added to 900 gm. of olive oil and 10 kg. of water. This emulsion is then applied to threads of cellulose and its derivatives to assist in processing operations such as weaving, spinning and knitting.

##### Example 10

20 1 lb. of the neutralized product of the reaction between castor oil,  $\text{P}_2\text{O}_5$  and ethylene glycol is added to 10 lb. of neat's-foot oil and the mixture applied to threads and filaments of cellulose and its organic derivatives such as cellulose acetate, to reduce friction in processing operations.

##### Example 11

25 30 5% of a neutralized phosphated castor oil prepared as described above is added to the common lubricants such as mineral oils, vegetable oils and blown oils to produce stable emulsions of the latter to facilitate their application to filaments and threads of cellulose and its derivatives, and their removal therefrom.

##### Example 12

40 45 3-10% by weight of the neutral reaction product obtained in Example 6 is applied by means of a wick, roll, or spray to threads or filaments of cellulose and its derivatives, to assist in textile processing operations.

##### Example 13

50 55 10% of the neutral reaction product between castor oil, cetyl alcohol and  $\text{POCl}_3$  worked up as previously described is applied to knitting yarn to reduce friction and electrification.

##### Example 14

Mixtures of any of the phosphated oils prepared above or similar ones are added to oils such as neat's-foot and applied to leather and leather substitutes to give softness and fine handle.

##### Example 15

100 gm. of reduced rapeseed oil are treated with



in a ratio of 1:1 in pyridine and the reaction completed by gentle warming. The solution is filtered and washed. The resultant waxy solid is insoluble in water.

##### Example 16

50 gm. of reduced castor oil are treated with 20 gm. of



in benzene and the HCl formed and benzene removed in vacuo. The reaction product is a low-melting waxy solid.

*Example 17*

100 gms. of unblown castor oil are heated with 40 grams of



at 40°-50° C. for 10 hours and then on a water bath for five hours. The product is cooled and poured into iced water containing sodium carbonate. It is found to be a water-soluble oil which has valuable properties as a wetting out agent, de-electrifier, and a lubricant in the treatment of yarns composed of or containing organic derivatives of cellulose.

*Example 18*

100 gm. of "blown" castor oil are heated at 100° with 24 gm. of sirupy phosphoric acid for 8 hr. and the product washed several times with water. The reaction product is a thick, dark colored, fluorescent oil which is soluble in water when neutralized with a base such as sodium or potassium hydroxides, ammonium hydroxide, ethylamine, triethanolamine choline, brucine, cyclohexylamine, etc.

*Example 19*

100 gm. of oxidized neat's-foot oil are heated with 70 gm. of 75% phosphoric acid at 60° for 8 hr. and the product washed with water several times and dried. The orange, viscous oil produced is soluble in water when neutralized with a base.

*Example 20*

50 gm. of oxidized olive oil are treated in the cold with 10 gm. of phosphorus pentoxide and 2 cc. of water. The reaction product is well washed with water and dried. The clear thick oil obtained is soluble in a basic solution.

*Example 21*

35 gm. of "blown" sperm oil are heated at 95° for 4 hr. with 10 gm. of sirupy phosphoric acid and 0.1 gm. of concentrated sulfuric acid. The heavy oily product is washed with water, dried under reduced pressure, and neutralized.

*Example 22*

500 gm. of blown rapeseed oil are treated with one equivalent of



in benzene and then warmed. The hydrochloric acid and benzene are removed under reduced pressure. The reaction product is hydrolyzed with dilute sodium bicarbonate. The acid phosphate may be neutralized with a base such as ditetrahydrofurfurylamine or diethylcylohexylamine to give a water-soluble compound.

*Example 23*

200 gm. of blown Japan wax are warmed with 50 gm. of  $\text{C}_{17}\text{H}_{35}\text{OPOCl}_2$  in chloroform. The chloroform and hydrochloric acid are distilled off under reduced pressure. The product is hydrolyzed and then neutralized with triethanolamine. It is a thick, yellow-brown, self-dispersible oil.

*Example 24*

5 A mixture of 33 gm. of blown teaseed oil, 33 gm. blown rapeseed oil, and 33 gm. blown peanut oil is treated with 140 gm. of  $\text{PSCl}_2(\text{NH}-\text{C}_{17}\text{H}_{35})$  in carbon tetrachloride and the reaction product worked up as previously described. The oil obtained is self-emulsifiable, stable to heat, and very viscous.

*Example 25*

10 A mixture of 75 gm. of blown neat's-foot oil and 25 gm. of blown carnauba wax is treated with 75 gm. of ethylene glycol and 20 gm. of phosphorus pentoxide. The reaction product is washed, dried, and neutralized. The semi-solid waxy material is fairly soluble in water.

*Example 26*

20 100 gm. of oxidized olive oil with a high acetyl value are treated with 10 gm. phosphorus pentoxide and 50 gm. methyl Cellosolve. The reaction product is neutralized with ditetrahydrofurfurylamine. The product is a resinous brown oil, fairly soluble in water.

*Example 27*

25 100 gm. of neat's-foot oil are blown in the presence of 20 gm. of sirupy phosphoric acid at 100° for 10 hr. The resulting product is water-soluble and resembles that obtained in Example 19.

*Example 28*

30 35 A mixture consisting of 50 ounces castor oil and 50 ounces blown kapok seed oil is heated with 20 ounces of 85% phosphoric acid and 6.7 ounces of phosphoric anhydride for 4 hr. The product is washed, dried and neutralized. It is a gelatinous, water-soluble oil.

*Example 29*

40 45 100 gm. of castor oil are heated with 60 gm. crystalline phosphoric acid until a jell is formed. The product is melted, washed with hot water and neutralized with an organic or inorganic base.

*Example 30*

50 55 100 gm. of blown and reduced neat's-foot oil are heated 10 hr. with 100 gm. of 75% thiophosphoric acid. The product is washed and neutralized.

*Example 31*

60 55 To 5 lb. of an anthraquinone dye are added 2 lb. of phosphated blown castor which has been previously almost completely neutralized, and the mixture is poured into water heated to 90°. 200 lb. of textile material in the form of thread or cloth are then dipped and dyed.

*Example 32*

65 70 1 lb. of a phosphated oxidized neat's-foot oil prepared as described above is added to 10 lb. of olive oil and 80 lb. of water. The emulsion is then applied to threads of cellulose and its derivatives to assist in processing operations such as weaving, spinning, etc.

*Example 33*

75 1 lb. of the neutralized product of the reaction between blown castor oil, phosphoric anhydride, and ethylene glycol is added to 10 lb. of neat's-foot oil and the mixture applied to threads of cellulose and its derivatives, especially cellulose acetate, to reduce friction in processing operations.

## Example 34

5% by weight of a neutralized phosphated castor oil-blown rapeseed oil mixture is added to the common lubricants such as mineral oil, vegetable oils, and blown oils to produce stable emulsions of the latter and facilitate their application to filaments and threads of cellulose and its derivatives, as well as to facilitate the removal of these oils therefrom.

## Example 35

1-5% of the neutral reaction product of blown olive oil, phosphorus oxychloride and Cellosolve is applied in the usual way to threads or filaments of cellulose and its derivatives to aid in textile processing operations.

## Example 36

85% of the neutral reaction product between castor oil, blown rapeseed oil and blown sesame oil is mixed with 15% of a softener such as glyceryl acetals, Cellosolve formal, glycols and polyglycols and ethers thereof. The mixture is applied to threads of cellulose and its derivatives to facilitate knitting operations.

## Example 37

Mixtures of any of the phosphates prepared above with oils such as neat's-foot oil are applied to leather to give softness and a fine handle.

## Example 38

10% of the neutral product of the reaction between blown carnauba wax,  $\text{POCl}_2(\text{OC}_{17}\text{H}_{35})$ , and cetyl alcohol is dissolved together with cellulose acetate stearate and 20% of a common plasticizer such as butyl or any phthalate, tri-phenyl phosphate, Cellosolve phthalate, etc. in a suitable solvent to produce a plastic of good strength, elasticity and appearance.

## Example 39

1% of a slightly acid phosphated oxidized castor oil is added to soap which is to be used in hard water.

## Example 40

A fugitive tint solution is prepared for application to textile threads, particularly of cellulose acetate, having the following composition:

|                                        | Grams |
|----------------------------------------|-------|
| Phosphated blown olive oil sodium salt | 0.2   |
| Blown olive oil                        | 2.0   |
| Chicago blue dye                       | 0.02  |
| Water                                  | 100   |

The emulsion is applied to the yarn by any suitable means such as a spray, wick, or roller and may be dried if desired.

## Example 41

|                                                  | Grams |
|--------------------------------------------------|-------|
| Phosphated blown castor oil triethanolamine salt | 5     |
| Blown neat's-foot oil                            | 20    |
| Dimethoxyethyl succinate                         | 75    |

## Example 42

|                                           | Grams |
|-------------------------------------------|-------|
| Phosphated blown corn oil morpholine salt | 2     |
| Mineral oil                               | 2     |
| Olive oil                                 | 5     |
| Ditetrahydrofurfuryl ether                | 10    |
| Water                                     | 300   |

## PHOSPHITED COMPOUNDS

## Example 43

37 g. of castor oil are added to 6 g. phosphorus trichloride in pyridine. The reaction is completed by warming. The product is filtered, treated with aqueous sodium carbonate. The reaction product is self disperible in water.

## Example 44

10 200 g. of rapeseed oil are warmed with 25 g.  $\text{PCl}_2$   
 $\text{HN}-\text{C}_{12}\text{H}_{25}$

15 and the reaction is completed by warming. The solution is filtered and the pyridine is removed under reduced pressure. The product is treated with water and then with ethylamine to give a viscous yellow oil.

## Example 45

20 Carnauba wax and phosphorus trioxide are heated in a molecular proportion of 1:1 on the steam bath for 24-60 hours. The product after neutralization with a suitable base such as diethylcyclohexylamine, ditetrahydrofurfurylamine, ethanolamine, etc., is self-disperible in water.

## Example 46

25 A mixture of 75 g. castor oil and 25 g. carnauba wax is treated with 70 g. phosphorus trioxide. The reaction product is neutralized with triethanolamine. The heavy brown oil forms an aqueous dispersion.

## Example 47

30 35 100 g. of reduced partly acetylated castor oil are treated at 50-100° for 10 hours with 60 g. phosphorus acid and 30 g. phosphorus trisulfide. The product is neutralized with tetramethylammonium hydroxide. The product forms an aqueous suspension.

## Example 48

40 45 200 g. Japan wax are treated with 200 g.  $\text{PCl}_2$   
 $\text{NH}-\text{CH}_3$

and worked up as above. The sodium salt is prepared.

## Example 49

50 55 100 g. blown castor oil are heated with 25 g. phosphorus acid at 110-115° for 5 hours with stirring. The product is then neutralized with triethanolamine and is soluble in warm water. In place of blown castor oil, we may use blown neat's-foot, sperm, olive, teased, soya bean, rapeseed, corn, menhaden, carnauba, Japan wax, etc.

## Example 50

60 65 100 g. blown neat's-foot oil are heated with 50 g. phosphorus acid as in Example 49 and the product is then treated in pyridine with 20 g. phosphorus trichloride. The reaction product is poured into dilute sodium hydroxide.

## Example 51

70 75 100 g. blown castor oil are reacted with 75 g. phosphorus acid as in Example 49 and then in pyridine with 20 g. phosphorus oxychloride. The diethylcyclohexylamine salt is made in the usual manner. The product is water soluble.

## Example 52

100 g. blown sperm oil are heated with a mixture of 40 g. phosphorus acid and 30 g. phosphoric

acid at 90-120° for 4 hours. The trimethylbenzyl ammonium hydroxide salt is water soluble.

*Example 53*

100 g. blown carnauba wax are reacted with 60 g. phosphorus acid as above.

*Example 54*

A mixture of 50 g. blown soya bean oil and 50 g. blown teaseed oil is reacted with 70 g. phosphorus acid as above and neutralized with a mixture of potassium hydroxide and dibutylamine.

*Example 55*

5 pounds 1,4-dimethylamino anthraquinone are finely ground with 2 pounds of the sodium salt of phosphited blown olive oil and poured into water heated to 85°. 200 pounds of cellulose acetate knit fabric are entered and dyed blue.

*Example 56*

1 pound of a phosphited oxidized neat's-foot oil is added to 10 pounds olive oil and 80 pounds water. The emulsion is then applied to threads of cellulose or its derivatives to assist in weaving, knitting, etc.

*Example 57*

5% by weight of a neutralized phosphated-phosphited castor oil-blown rapeseed oil mixture is added to lubricants such as mineral oil and blown and unblown vegetable and animal oils to produce stable emulsions of the latter and to facilitate their application to filaments, threads and the like composed of cellulose and derivatives, including regenerated cellulose.

As indicated by the above examples, the phosphated and phosphited blown and unblown oils, fats, or waxes of our invention may be employed with a high degree of effectiveness as emulsifying, wetting out and deelectrifying agents in the compounding of yarn treating compositions. Various ingredients such as other lubricating agents, solvents, non-solvents, blending agents and the like may be employed in connection with these compounds within the scope of our invention. Likewise, various dyes or other coloring matter may be employed in case it is desired to permanently or fugitively tint or dye the material undergoing treatment.

Although we have found it convenient to illustrate our invention by reference to compositions containing specific percentages of the various ingredients, these percentages may vary widely depending upon the particular purpose for which the composition is intended.

While we have described our invention with reference to the preparation of emulsions particularly adapted for the treatment of yarns composed of organic derivatives of cellulose such as cellulose acetate, the broad scope of our invention includes the preparation of emulsions adapted for the treatment of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted

together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

What we claim is:

1. The process of simultaneously lubricating and eliminating the tendency of yarns, filaments or fibers composed of or containing organic derivatives of cellulose to accumulate charges of static electricity, which comprises applying thereto a composition containing as its essential lubricating and anti-static component an oil which is the product of reaction obtained by first blowing an oil containing compounds having a certain degree of unsaturation to produce compounds having at least one free hydroxyl group or its equivalent in its molecule which is subject to phosphation or phosphition, and then reacting the blown oil with an agent selected from the group consisting of phosphating and phosphiting agents.
2. The process of simultaneously lubricating and eliminating the tendency of yarns, filaments or fibers composed of or containing organic derivatives of cellulose to accumulate charges of static electricity, which comprises applying thereto a composition containing as its essential lubricating and anti-static component a phosphated oil which is the product of reaction obtained by first blowing an oil containing compounds having a certain degree of unsaturation to produce compounds having at least one free hydroxyl group or its equivalent in its molecule which is subject to phosphation, and then reacting the blown oil with a phosphating agent.
3. The process of simultaneously lubricating and eliminating the tendency of yarns, filaments or fibers composed of or containing cellulose acetate to accumulate charges of static electricity, which comprises applying thereto a composition containing as its essential lubricating and anti-static component a phosphated oil which is the product of reaction obtained by first blowing an oil containing compounds having a certain degree of unsaturation to produce compounds having at least one free hydroxyl group or its equivalent in its molecule which is subject to phosphation, and then reacting the blown oil with a phosphating agent.
4. The process of simultaneously lubricating and eliminating the tendency of yarns, filaments or fibers composed of or containing organic derivatives of cellulose to accumulate charges of static electricity, which comprises applying thereto a composition containing as its essential lubricating and anti-static component a phosphited oil which is the product of reaction obtained by first blowing an oil containing compounds having a certain degree of unsaturation to produce compounds having at least one free hydroxyl group or its equivalent in its molecule which is subject to phosphition and then reacting the blown oil with a phosphiting agent.
5. The process of claim 2 in which the phosphated oil is phosphated blown neat's-foot oil.
6. The process of claim 2 in which the phosphated oil is phosphated blown olive oil.
7. The process of claim 2 in which the phosphated oil is phosphated blown sperm oil.

JOSEPH B. DICKEY.  
JAMES G. McNALLY.